

## UNITED STATES PATENT OFFICE

FREDERICK KNÄPP FISH, JR., OF SAN FRANCISCO, CALIFORNIA.

## PROCESS OF PREPARING PAPER PULP.

No Drawing. Application filed May 24, 1926, Serial No. 111,368, and in Canada July 7, 1925.

This invention relates to a process of treating wood for the production of pulp and more particularly to the treatment of the wood after it has been chipped.

5. In other applications for Letters Patent, I have described certain processes for the treatment of plant material in which solvent extractives of the material are used in the processes for attacking the binding and 60 intercellular constituents of the material in order to liberate the fibre, both with and without the addition of further chemical reagents.

10. The present invention relates to a further development in the art of producing pulp and has for its main object the reduction of the cost of the production of pulp of a standard or improved quality.

15. I have found that the addition of sulphur to the liquor applied to the chips produces very desirable results in hastening the cook and in some manner, which I am unable at present to fully explain, improves the condition of the fibre of the cooked material and 20 the color of the pulp produced therefrom.

25. In carrying out my process the chips are charged into the digester where they are treated with a liquor to which sulphur is added. The liquor is preferably initially charged with volatile and other solvent extractives of wood and the desired chemical reagent, such as soda, caustic potash, lime and the like is added. The sulphur may be dissolved directly in the liquor or it may be 30 previously dissolved in a suitable solvent and then added to the liquor. I have found it satisfactory in some treatments to charge the sulphur directly into the digester prior to or during the period of supplying liquor 35 to the charge. In such cases the sulphur appears to be distributed through the contents of the digester, to dissolve in the liquor and otherwise act on the chips to effectively treat the same so as to soften, dissolve and remove 40 or distribute the resins, lignin and other constituents which surround the wood fibre so that the cooked charge is in the desired 45 condition for further treatment.

50. During the charging operation the liquor is preferably circulated and sprayed on the chips to assist and hasten the saturation of the chips with the liquor. When the digester is completely charged a vacuum is produced therein to remove air from the charge and a 55 vacuum of 15 or 20 inches is maintained for

a limited period. During this stage of the process the circulation and spraying of the liquor is preferably continued. The full charge of liquor is then admitted to the digester and the temperature is raised to complete the cook. 60

I have thus been enabled to considerably reduce the time required for cooking the wood and the pulp produced has a tough fibre and improved color. 65

While as previously stated I am not prepared to assign a definite reason for the beneficial results by the treatment herein described, it is to be noted that the reactions between the sulphur and other constituents 70 of the liquor take place in contact with or in the wood chips and all of the products of reaction are thus free to act on the binding constituents of the wood fibre. With liquors prepared prior to charging the same into 75 the chips in the digester the reactions mentioned do not take place in contact with the chips. It is possible that this may be to some extent responsible for the improved results obtained, but obviously I do not wish 80 to limit this invention to any particular theory which may underlie the operation of the process.

## What I claim is:

1. A process of producing pulp which 85 consists in cooking chips in a digester with a liquor containing solvent extractives of plant material to which sulphur has been added.

2. A process of producing pulp which 90 consists in cooking chips with a liquor charged with volatile and other extractives of plant material and in which sulphur is incorporated.

3. A process of producing pulp which 95 consists in treating chips in a digester with a liquor containing a chemical reagent and extractives of plant material in which sulphur is dissolved.

4. A process of producing pulp which 100 consists in adding sulphur to the charge of chips in a digester, circulating liquor containing extractives of wood in the charge and cooking the chips therewith.

5. A process of producing pulp which 105 consists in adding elemental sulphur to the chips in a digester and cooking the same with a liquor made from sodium carbonate and lime.

6. A process of making pulp which 110

sists in cooking chips in a digester with a liquor initially containing elemental sulphur, solvent extractives of wood and an alkali and utilizing in the cook, products of the reaction between the sulphur, alkali and extractives, said products being formed in contact with the chips.

7. A process of producing pulp comprising treating the chips in a digester in the presence of the reaction between elemental sulphur, chemical reagent which will unite with the sulphur, and added extractives of wood, the sulphur reagent and extractives being free to react with or on the binding

constituents of the chips during the progress 15 of the reactions.

8. A process of producing pulp comprising mixing elemental sulphur with a chemical reagent in the absence of air and treating chips in a digester with liquor so produced and maintained free from atmosphere to cause such liquor to react with the binding constituents of the chips to so act on the chips as to permit the liberation of the fibre in the cook. 20 25

In testimony whereof I affix my signature.

FREDERICK KNAPP FISH, JR.